

Aug. 14, 1928.

**1,680,497**

H. E. BROWN ET AL.

# IMPREGNATED FABRIC AND PROCESS OF MAKING THE SAME

Filed Sept. 7, 1922

2 Sheets-Sheet 1



Norman E. Brown Inventor,  
and Jordan Homer Storer  
By their Attorney  
Louis Prevost (Signature)

Aug. 14, 1928.

1,680,497

H. E. BROWN ET AL

IMPREGNATED FABRIC AND PROCESS OF MAKING THE SAME

Filed Sept. 7, 1922

2 Sheets-Sheet 2

Fig. 6.



Herman E. Brown Inventor  
and Jordan Horner Stoer, Inventor  
By their Attorney  
Louis Prevost Whitaker

Patented Aug. 14, 1928.

1,680,497

# UNITED STATES PATENT OFFICE.

HERMAN E. BROWN, OF KINGSTON, NEW YORK, AND JORDAN HOMER STOVER, OF NUTLEY, NEW JERSEY, ASSIGNEES, BY MESNE ASSIGNMENTS, TO RESPRO INC., OF PROVIDENCE, RHODE ISLAND, A CORPORATION OF RHODE ISLAND.

## IMPREGNATED FABRIC AND PROCESS OF MAKING THE SAME.

Application filed September 7, 1922. Serial No. 386,803.

Our invention, which is a continuation in part of application No. 493,526, filed Aug. 19, 1921, consists in the novel features hereinafter described, reference being had to the accompanying drawings, which illustrate diagrammatically a form of apparatus which may be advantageously employed in carrying our process into effect, and the said invention is fully disclosed in the following description and claims.

The object of our invention is to treat a fibrous fabric in which the fibres exist in a more or less loosely associated relation, the fibres being preferably unspun, unwoven natural fibres arranged in a flat form, as cotton batting, for example, or in a felted condition, as in cotton felt, for example, with a binding material, preferably waterproof and preferably a rubber compound, in the form of a semi-solid, that is to say, a dough or putty like form and plastic at the time of application, as distinguished from a so-called solution in which the binding material is dispersed in a more or less volatile liquid, and as distinguished from a material in a fluid or molten condition, and to mechanically force, by the application of pressure under the proper conditions of temperature, the said binding material uniformly into the fabric so as to coat the individual fibres throughout the entire fabric without completely filling the interfibre spaces, and uniting the fibres of the fabric by the cohesion of their individual coatings at points of contact and intersection, and in some instances by additional bonds from one fibre coating to another so as to produce a resulting fabric which, when dried, cured or vulcanized, closely resembles leather, and is suitable for many of the purposes for which leather is used. Where the binding material is a rubber composition and is thereafter properly vulcanized to convert it from the plastic to the elastic form, the resulting fabric possesses elasticity in all directions, due to both the elastic quality of the binding material, which unites the fibres yieldingly at their points of intersection and bonding contact, and the fact that the interfibre spaces are not completely filled, which permits relative movement of the fibres with respect to each other, and contributes to the elasticity of the fabric as ordinarily produced. The resulting fabric is pervious to

air and dry gases, by reason of the minute unfilled spaces between the fibre coatings, while it is practically impervious to water, owing to the fact that these interfibre spaces are so minute and the repellent action of the binding material is such, that water does not pass through in the absence of pressure, and the fabric will not materially absorb water, as the coating of the individual fibres prevents the penetration of water thereinto. We are aware that attempts have been made to treat the fibrous material by the application thereto of binding material in liquid form. Where a liquid mixture is employed, the amount of liquid solvent or dispersing agent is from ten to twenty times the bulk of the rubber or other binding material dissolved or dispersed therein. Even if the fabric is thoroughly penetrated by such a liquid, the drying out or evaporation of the liquid would leave not more than from five to ten per cent of the absorbed liquid, as solid matter (rubber for example) distributed among the fibres of the fabric, too little to effect either the coating of the fibres, or the adequate binding of them together. As a matter of fact, the amount of binding material left in the fabric is even less than would be expected, as rubber for example has a greater cohesion than adhesion and where a fabric has been treated with a liquid rubber mixture and subjected to drying action, the liquid mixture within the fabric flows from the interior of the fabric toward the exterior in drying, thus actually withdrawing the solution or mixture, as a mixture, and including both the solvent and the dispersed rubber from the interior to the exterior of the fabric in a manner somewhat similar to that resulting where a porous material, such as a brick, is saturated with a solution of a chemical solid and on drying the brick the dried solid is deposited, largely, if not entirely, at or upon the exterior surface of the brick. We have found it to be a fact, by microscopic examinations, that where fibrous material of appreciable thickness is treated with such liquid mixture, there is little, if any, of the binding material (rubber) left in the interior of the fabric, and what small amount of the rubber solution absorbed by the fabric remains in the fabric, on the drying will be found at or upon the surface fibres of the fabric, the

central portion of the fibres being practically bare, uncoated and not united by the binding material. Where any rubber or other binding material is left among interior fibres, it tends to collect in minute globules, and owing to its cohesion, it draws itself together and away from the fibres, leaving the interior fibres naked and uncoated. Where the fibres cross each other or come in contact, they do not adhere to each other and are not united or bound together. Where they cross each other, a sharp line of crossing is noted under the microscope showing the bare fibres unattached. Moreover where fibrous material is treated by the liquid process it is extremely difficult if not impossible to carry materials insoluble in the dispersing liquid, such as oxide of zinc, whiting, magnesium oxide, sulphur, coloring compounds, etc., into the interior of the fabric, as the fibrous material of the fabric acts in the same manner as a filter cloth in a filter press, to hold back such solid insoluble matters and prevent them from passing through into the fabric, thus leaving them on the outer surface.

In some instances it has been proposed to wring out or squeeze a liquid treated fabric between rollers or otherwise, but it will readily be seen that as this squeezing treatment removes a large percentage of the liquid mixture which has penetrated into the fabric, the resulting amount of solid binding material left in the fabric when it is dried, is correspondingly reduced, and in fact is extremely minute. In accordance with our invention, we take a fibrous material, preferably composed of unspun, unwoven fibres, such as cotton felt, cotton batting and the like, for example, or any material made from natural fibres, and treat the same with binding material, preferably rubber compounds or plastic compositions, for example, in a semi-solid form, that is to say in a dough like or putty like mass of such composition and consistency, and plastic at the time of application, as to be capable of penetrating into the interfibre spaces of the fabric, and uniformly coating the fibres thereof, without filling completely the interfibre spaces, and leaving the fibres coated at their points of intersection and contact by the cohesion of the individual fibre coatings, and in some instances connected by additional bonds of the binding material between the fibre coatings. The material is preferably and ordinarily applied by the application of pressure, and preferably between calender rollers, the temperature and relative speeds of which are maintained in such a manner, according to the composition of the binding material employed as to effect the stated result. The fibres as they pass between the calender rolls are compressed beyond a point at which they will be held in position by the plastic semi-

solid binding material in its then condition, forced into the fabric, and on the release of pressure, the fibres, by their inherent elasticity, tend to expand slightly and rearrange themselves, so as to form minute interfibre spaces, unfilled by the binding material, which is later set by the drying, curing or vulcanization of the resulting fabric.

We believe that we are the first in the history of the art to impregnate a non-woven material composed of unspun non-twisted and non-woven fibres by forcing thereinto a binding material in semi-solid condition, plastic at the time of application, and we believe that we are the first to accomplish this result by means of calender rolls.

Referring to the accompanying drawings,

Fig. 1 is a form of apparatus which may be conveniently employed in carrying our process into effect.

Fig. 2 is a diagrammatic view illustrating a form of apparatus which may be conveniently employed where the fabric is treated first from one side and then from the other, with or without a final rolling to insure both sides of the fabric being smooth.

Fig. 3 is a diagrammatic sectional view illustrating the effect of the process on the fabric where the binding material is forced entirely through the fabric, leaving one surface of the fabric in a slightly roughened condition with upstanding coated fibres to serve as bonds for an exterior coating.

Fig. 4 is a similar view to Fig. 3 illustrating the effect on the fabric where the binding material is applied to one face and forced partly but not entirely through the fabric.

Fig. 5 is a view similar to Fig. 3 illustrating the completed fabric after a subsequent rolling operation, to smooth down the roughened surface and upstanding fibres left by a preceding application of the binding material.

Fig. 6 is a view greatly magnified illustrating actual fibres from the interior of the fabric as they appear under the microscope and illustrating more or less graphically the fibre coatings connected at their points of intersection and contact and additional bonds of the binding material connecting the fibre coatings.

As illustrative of our improved process, the following example is given of a specific binding material, and the specific manner in which it is applied to produce our improved fabric. In this example, we use a composition consisting of

250 parts of washed and dried guayule rubber,  
250 parts of smoked rubber sheets,  
450 parts of zinc oxide,  
25 parts of washed and dried flowers of sulphur,  
15 parts of mono-chloro-naphthaline.

In preparing this compound the smoked sheets are first broken down or macerated on a mixing mill, as regularly employed in the rubber industry, by milling until the 5 rubber is partially or wholly denerved, which quality can be detected by pulling a piece of milled rubber apart between the fingers and observing the manner in which it separates, the denerving of the rubber being sufficiently complete when it pulls apart 10 without the appearance of any lumps in the attenuated portions. The broken down sheets are then removed from the mill and the guayule rubber is placed on the mill and 15 warmed by working. The broken down sheets are then added to the guayule rubber and then the mono-chloro-naphthaline is added, and the mixture milled until it has a uniform consistency and color. The zinc 20 oxide and the sulphur are then added and mixed until they are uniformly distributed throughout the mass. It will be noted that the materials above mentioned are brought into the semi-solid plastic condition without 25 the use of volatile solvent, such as are employed in making so-called rubber solutions or cements. The mono-chloro-naphthaline is an oily material not volatile, the addition of which facilitates the softening and working 30 of the rubber without injuring its quality or burning it, which might otherwise result unless the operations were most carefully watched, to prevent undue heat.

The compound is then transferred to a 35 warming mill preparatory to feeding the calender upon which the compound is to be forced into the unwoven fibrous fabric. The mixing mill and calender may be machines of standard approved types as used extensively 40 in the rubber industry, in the manufacture of friction tire fabrics. Such a calender is illustrated in Fig. 1 of the drawing, in which 1, 2 and 3, represent a vertical series of three rollers provided internally with independent 45 heating means which may be of any usual or desired character, and in this instance is indicated as a heating coil arranged within each of said rollers, said coils being indicated by the numerals 4, 5 and 6, which are connected with pipes 7, 8 and 9 respectively, passing through the supporting trunnions of the 50 rollers. The central roller, 2, is supported in stationary bearings and the upper and lower rollers 1 and 3 in vertically adjustable 55 bearings provided with any desired type of adjusting means by which variable pressure may be applied. In this instance the bearings for the rollers 1 and 3, indicated at 10 and 11 respectively, are shown as provided 60 with adjusting screw shafts 12 and 13 respectively, which can be operated by hand wheels, or in any other desired manner. The rollers 1, 2 and 3 are provided with means for regulating independently the temperature of 65 each, which temperature adjusting means

can be of any usual or desired character. In the present instance we have shown a steam pipe, indicated at 14, and a cold water pipe indicated at 15, arranged vertically on opposite sides of the trunnions of the vertical series of rollers, each of said pipes being connected with the inlet pipes 7, 8 and 9, leading to the temperature regulating coils within the rollers, and each of the branch pipes is provided with an independent controlling valve. The branch pipes for the roller 1 are indicated at 16 and 17, and the valves therefor, at 18 and 19 respectively. The branch pipes for the roller, 2, are indicated at 20 and 21, and the valves therefor, 25 at 22 and 23 respectively. The branch pipes for the roller, 3, are indicated at 24 and 25, and the valves therefor, at 26 and 27 respectively. The rollers are so geared that the center roller moves at a considerably faster 30 speed than the others. The differential in speed of the center roller which we have found most suitable for the material given above is that of about three to one.

The calender is provided with the usual feeding and rolling up devices (not shown) for the fabric. In treating the fabric, the binding compound, in the form of a dough like or putty like semi-solid and plastic at the time of application, is applied from the warming mill to the calender between the top roller, 1, and the central roller, 2, as shown at 28. The temperatures of the various rollers are adjusted so that the mixed, milled compound adheres in a thin sheet to the central roller and does not adhere to the top roller. The bottom roller is well heated with dry steam to the desired temperature. A few small strips of the cotton felt or other fibrous material to be treated, in which the fibres are in a more or less loosely associated condition, are first thoroughly dried, and are then passed through the calender between the central roller, 2, and lower roller, 3, with such adjustments of the upper and bottom 100 rollers that the binding material is pressed into the fabric so as to uniformly coat the fibres without completely filling the inter-fibre spaces and leaving the fibres united by the cohesion of their individual coatings at 105 their points of contact and intersection. The pressure of the rollers compresses the fibres beyond the point at which they will be held by the binding compound in its then plastic condition, and the binding material is forced 110 into the fabric, as above described so as to substantially uniformly coat the fibres. When the pressure is relieved as the fabric leaves the calender rolls, the fibres expand somewhat by their inherent elasticity and 115 form inter-fibre spaces between the coatings, leaving the coatings connected at their intersections and points of contact and also in many instances forming additional bonds of binding material connecting said fibre coat. 120

ings. This will, of course, depend somewhat upon the weight and compactness of the fibrous material used. Where a cotton felt having a weight of four and a half ounces per square yard is employed, an adjustment of the top and bottom rollers with respect to the central roller, so that a bank of the binding material is formed over the felt as it is entering between the center and top rollers with a bank thickness of from one eighth to one quarter of an inch, is found to give very good results. After the proper adjustment of the calender has been determined by the use of strips or pieces of the fabric, so as to secure the desired result, a continuous length of the unwoven fabric is drawn from a roll and passed through the calender. The supply of binding material is maintained by periodic additions of the prepared material from the warming mill. The weight of the finished goods is about twelve ounces per square yard. Where, for operating purposes, it is not desired to maintain the calender at such accurate adjustments, or where extra heavy goods are run, the goods may be passed through on one side and the binding material forced somewhat past the middle point, and then run through on the opposite side to complete the coating of the fibres and their union by the cohesion of their coatings, without completely filling the interfibre spaces.

As the fabric leaves the roller, 2, on the side opposite that from which it enters, the separation of the fabric from the layer of binding material, 29, on the roller, 2, leaves the surface of the fabric adjacent to the roller, 2, slightly roughened, and the binding material being slightly tacky, any loose fibres on the surface, which are of course thoroughly coated, will be left in a more or less vertical position, perpendicular to the surface of the fabric, as indicated diagrammatically in Figs. 3 and 4, and these upstanding coated fibres will form bonds for firmly uniting to the fabric subsequently any surface coating which it may be desired to apply thereto, as where the fabric is employed as a base fabric in the manufacture of artificial leather and the like. Fig. 3 is a diagrammatic representation of the fabric as produced where the operation is so conducted that the binding material is caused to uniformly coat all the fibres throughout the material in a single pass or operation. The surface adjacent to the roller, 2, is indicated as a roughened surface, at 32, and the upstanding coated fibres are diagrammatically indicated at 33. Fig. 4 is a similar diagrammatic sectional view illustrating the fabric after it has been treated under conditions of speed and pressure, such that the binding material is caused to coat the fibres substantially half way through the thickness of the fabric, the

roughened surface adjacent to the roller, 2, being indicated at 34, and the upstanding fibres at 35. Where the process is carried out in this manner, the fabric is reversed and given another pass through the same or another similar apparatus, so as to force the binding material into the reverse side of the fabric, and coat the fibres of the remaining portion, in which case the roughened surface, 34, and upstanding fibres, 35, of the previously coated surface, will be rolled down by contact with the smooth roller, 3, and the last treated side of the fabric will be left with a roughened surface and upstanding fibres, as indicated in Fig. 3. If it is desired to have the fabric perfectly smooth on both sides, this can be readily accomplished by passing the fabric through a pair of plain rollers to roll down the roughened surface and upstanding fibres on the face last treated, leaving the fabric in the condition illustrated diagrammatically in Fig. 5.

In Fig. 2 we have illustrated diagrammatically, apparatus for treating the fabric on both sides by continuous operation. In this instance the fabric is first passed through an apparatus of the kind described, comprising rollers, 1, 2, 3, for the purpose of coating the fibres substantially half the thickness of the material, after which it is turned and passed between the proper rollers of another series of rollers, 1<sup>a</sup>, 2<sup>a</sup> and 3<sup>a</sup>, constructed and operated in the same manner as hereinbefore described, the fabric being turned in any usual manner, as by means of vertical guiding rollers, indicated at 36. Where it is desired to have the fabric entirely smooth on both sides, the fabric, indicated at 31<sup>a</sup>, may be passed between plain rollers 37 and 38, as indicated in Fig. 2, to roll down the face last treated, and leave the fabric in the condition indicated in Fig. 5, but where a surface coating of any kind is to be applied to the fabric, it will be found distinctly advantageous to use it in the form indicated in Fig. 3.

The goods may be cured in rolls between sheeting upon drums in an autoclave at the following cure:— fifteen minutes at ten pounds open steam pressure, and an hour and a quarter at twenty pounds open steam pressure. When cured in the press, the goods should be cured for thirty five minutes at fifty pounds steam pressure in the steam jacket. The foregoing example states only one of a number of compounds which may be utilized in carrying our process into effect. With other compounds containing other grades of rubber than those mentioned above, along with asphaltum, mineral rubber substitute, Burgundy pitch, pasty substitute, brown and white factice, with various mineral fillers, such as litharge, whiting, barytes, antimony sulphide, sienna, and

- other inorganic and organic accelerators and dispersing agents, variations in the calender adjustments and cure will be required in line with general practice in the handling of such compounds as may be constructed. It is obvious that by varying the composition of the binding material, a wide range of properties of the resulting fabric can be obtained.
- 5 10 The application of the binding material in dough like semi-solid condition by the aid of pressure, in the manner described, compresses the fibres so as to drive out the occluded air and permit the binding material to penetrate thoroughly and thoroughly coat the fibres through the entire thickness of the fibrous material treated. As the pressure is relieved, there will ordinarily be a slight expansion of the fibrous material, due to the resiliency of the fibres. This causes the coated fibres to adjust themselves and separate slightly, but leaves them connected by the cohesion of their coatings at separated points, accumulations or agglomerations of the binding material resulting at their various intersections or points of contact, and frequently additional bonds extend between the fibre coatings, which are plainly visible under the microscope, and when the resulting fabric has been hardened, cured or vulcanized, as the case may be, a fabric of great tensile strength results. Thus, in Fig. 6, which illustrates a number of fibres taken from the central portion of our improved fabric and magnified, 40, represents the fibres, 41, the coatings thereof, connected at points of intersection and contact, as at 42, by the cohesion of the fibre coatings and 43, represent additional bonds 30 of the binding material connecting the coatings of individual fibres.
- An examination of our improved fabric under a microscope shows it to have an almost uniform quasi-crystalline appearance, all of the fibres being thoroughly coated and bound together by the cohesion of their coatings, and by bonds connecting the fibre coatings, without filling completely the inter-fibre spaces, thus forming minute and substantially uniform interstices between the coatings of the fibres at points between the intersections and points of contact of said fibre coatings, and between said bonds throughout the material. Our fabric, therefore, is clearly distinguished from fabrics in which fibrous material is incorporated in a solid mass of rubber or other plastic produced by mixing and vulcanizing rubber or like material and causing it to solidify through and around the incorporated fibres or otherwise. In contra-distinction to this type of fabric our improved fabric is actually pervious to air and dry gases and is necessarily much lighter and more flexible than those fabrics in which a solid body of
- 5 35 40 45 50 55 60 65 70 75 80 85 90 95 100 105 110 115 120 125
- colloidal material surrounds incorporated fibres. At the same time our improved fabric, while pervious as before stated, to air and dry gases, is substantially impervious to water and many other liquids and is practically waterproof. We understand this apparent contradiction to be due to the fact that the fibres of our improved fabric are thoroughly and individually coated with the binding material so that they cannot absorb water, and the apertures or interstices between the adjacent fibre coatings are so minute and the repellent action of the binding material of the fibre coatings to water is so great that the water remains on the surface in somewhat the same manner as quicksilver will remain for the same reason on the surface of a piece of chamois leather, which air and dry gas will readily penetrate. A sheet of our improved fabric has been suspended horizontally and the convex portion filled with water and permitted to remain for ten or twelve hours without apparent absorption of water into or penetration of water through the fabric. It will be readily understood that this peculiar and novel characteristic of our improved fabric fits it admirably, for purposes of clothing, on account of its extreme lightness and flexibility, its water-proofness and its ventilating or "breathing" qualities. Another highly important feature of our new fabric is that when rubber is used as the binding material, it is elastic or yielding in all directions due in part to the fact that the fibres are in a slightly spaced or open relation, and partly to the fact that they are held yieldingly at their points of contact and intersection by the union of the fibre coatings which are in themselves elastic when the material has been vulcanized so as to convert the plastic binding material into the elastic condition. Both factors co-operate in permitting the fabric to be elongated in any direction and to resume its normal condition. This characteristic of our new fabric makes it particularly desirable as a substitute for leather or as a base fabric for leather substitutes. Cushions and other upholstery covered with our fabric will yield to pressure and resume their original form without producing wrinkles which are soon formed in the ordinary leather substitutes, which, not being elastic, are soon stretched so as to produce a sag or looseness in the coverings. Our new fabric can be used with great advantage for waterproof clothing, for the uppers as well as for the soles and heels of shoes (in the case of soles and heels a number of superimposed layers of the fabric being employed and consolidated by the binding material), in all of which its elastic character is desirable, as well as for tarpaulins tents, boat covers, and all purposes where a light and waterproof material is desired.

- It also forms an admirable substitute for leather, and if desired, can readily be made entirely impervious, either by subjecting it to great pressure, or by the application thereto of any of the usual or preferred types of coatings, such as varnish, the usual cellulose nitrate and cellulose acetate coating compositions, for example, or any other preferred coating compositions.
- 10 If a denser or heavier fabric is desired, we can readily produce the same by adding to the dough like or putty like rubber compound, or other binding material used, a desired preparation of solid insoluble material, such as, for example, oxide of zinc, whiting, magnesium oxide, sulphur oxide, and various coloring compounds, antimony sulphide, oxides of iron, gas black or lamp black, and various pigments which can be 15 forced mechanically, as before described, into the interior of the fabric with and after having been thoroughly incorporated in the dough like binding material, thereby imparting any desired degree of density, 20 thickness, weight, shade or color to the resulting fabric uniformly throughout the thickness thereof.
- Our fabric can also be made denser and substantially, and in some cases, wholly impervious, by subjecting it to great pressure sufficient to force the fibre coatings and fibres together and substantially close the interstices or interfibre spaces which would otherwise exist. This may be accomplished 25 by subjecting a single sheet or a series of superimposed sheets, united by a rubber compound or other binding material, or cement, to great pressure, as in a hydraulic press, and such highly compressed material 30 may or may not be vulcanized, as desired. Shoe soles and heels can be formed in any desired thickness in this manner, and would be impervious, and at the same time both flexible, and to an extent elastic, al- 35 though not so elastic as the material formed without the use of this increased pressure treatment. Belting and straps can also be formed in this way, also floor coverings and like sheet materials.
- 40 Our improved fabric can be given any desired color either by mixing pigments with the binding material, or otherwise. It can be used either with or without a surface coating for book covers and many other uses where leather or imitation leather is now employed, and its elastic character adapts it especially for such purposes, and for up- 45 holstery, automobile tops, etc., where it is stretched over unelastic surfaces or frames.
- 50 In the preparation of our improved fabric it may or may not be vulcanized after treatment, as before described. With the binding material such as described, we prefer to subject it to a drying, curing or vulcanizing action by any of the well known

methods for treating such materials, such for example, as the festooning method, the curing chamber method, the autoclave method, or any other desired manner for the purposes of drying, curing or vulcanizing it.

While our improved fabric is substantially impervious to water in that it will not permit the passage of water therethrough, nor will the coated fibres absorb water, 75 we have found that a slight amount of moisture may be deposited in the interstices or interfibre spaces adjacent to the face of the fabric, especially if the fabric is subjected to pressure. For example, we 80 have found by experiment that our new fabric is peculiarly suitable for use for the sweat bands of hats, and is much more desirable than a glazed imitation leather. When so used, the moisture of perspiration, instead of running down the band, upon the forehead, is held in the surface interstices of the fabric, and when the hat 85 is removed, the moisture quickly evaporates on account of the permeability of the material to dry air. Where an elastic material is desired, the material is preferably vulcanized in such manner as to convert the binding material from the plastic to the elastic condition, and impart the desired degree 90 of elasticity to the finished material.

We are of course aware of the fact that calenders have been used for applying surface and so-called friction coatings to woven fabrics, and that in some instances the material of such surface coatings has been caused to enter between the crossed warp and weft threads, in substantially the same manner that plaster is pressed through supporting laths. In such instances, however, 100 there is no coating of the fibres of the material, and on cutting such a material, the fibres of which the threads are composed will be found to be in their natural condition and the interior fibres uncoated and 105 out of contact with the coating material.

We believe that we are the first to apply to a fabric in which the fibres are in a more or less loosely associated relation, a binding material in a semi-solid condition and plastic at the time of application, which we have referred to as a dough like or putty like condition, so as to cause it to coat the fibres without filling completely the interfibre spaces and leaving the individual fibres connected by the cohesion of their coatings at points of contact and intersection, and we believe ourselves to be the first to apply a binding material to a non-woven fabric by means of a calender. It is extremely im- 115 portant that the binding material be in the proper condition in order that it may be caused to penetrate into the fabric and coat the individual fibres in the manner described. The composition must have a high degree of 120

- cohesion and also a high degree of adhesion, so that while it tends to cling to itself, it will also cling around and coat the individual fibres. The condition of the binding material may be aptly described as being substantially that of a rubber base chewing gum which has been chewed at the temperature of the human body. According to our process we force into the fabric much greater 10 quantities of our binding material than can be possible or has ever been attempted to be, accomplished by the wet process, which is the only method of impregnation heretofore effected. It has heretofore been considered 15 impossible to impregnate an unwoven fabric in any other way than by the wet process, and we have demonstrated that this can be successfully accomplished by our improved process. The increase in weight of our im- 20 proved fabric after impregnation in the manner described herein is from  $1\frac{1}{2}$  to 3 times that of the original fabric, and the process may be carried out by a single pass of the material through the roll, or if pre- 25 ferred, by not more than two passes.

We are aware of the fact that woven fabrics have been coated or frictioned with binding material, which is applied by means of a calender, but these processes have no 30 bearing whatever on our process, and there is not the slightest resemblance between our improved fabric and the coated and frictioned woven fabrics produced by the old calendering methods. In the case of coat- 35 ings, the coating material is usually applied in a very thin, almost liquid condition, and spread upon the surface of the woven fabric. In the case of friction tire fabric and the like, and in the manufacture of linoleums, 40 the plastic material used is pressed upon the woven fabric and will naturally extend into or through the orifices between the warp and weft threads, but this is entirely different from our process, as the plastic used in such 45 frictioning and calendering processes merely extends part way around the twisted threads without penetrating into the interior thereof and without coating the individual fibres of the fabric at all.

50 What we claim and desire to secure by Letters Patent is:—

1. The herein described process, which consists in applying to a fabric composed of unspun unwoven natural fibres, a binding material in the form of a dough like semi-solid plastic at the time of application, having such high cohesiveness and adhesiveness as to be capable of penetrating around and between the natural fibres, and forcing said 55 binding material by pressure into the fabric and around and upon the individual fibres so as to coat the individual fibres throughout the fabric without completely filling the interfibre spaces and causing the fibres to adhere at points of contact and intersection

by the cohesion of their individual coatings.

2. The herein described process, which consists in applying to a fabric composed of unspun unwoven natural fibres, a binding material in the form of a dough-like semi- 70 solid and plastic at the time of application, having such high cohesiveness and adhesiveness as to be capable of penetrating around and between the natural fibres, and forcing said binding material by pressure into the 75 fabric and around and upon the individual fibres so as to coat the individual fibres throughout the fabric without completely filling the interfibre spaces and causing the fibres to adhere at points of contact and in- 80 tersection by the cohesion of their individual coatings, and treating the resulting fabric so as to convert the binding material into an elastic material.

3. The herein described process, which consists in applying to a fabric composed of unspun unwoven natural fibres, a vulcanizable binding material in the form of a dough like semi-solid plastic at the time of applica- 85 tion, and having such high cohesiveness and adhesiveness as to be capable of penetrating around and between the natural fibres, and forcing said binding material by pressure into the fabric and around and upon the individual fibres so as to coat the individual 90 fibres throughout the fabric without com- 95 pletely filling the interfibre spaces and caus- ing the fibres to adhere at points of contact and intersection by the cohesion of their in- dividual coatings, and vulcanizing the re- 100 sulting fabric so as to change the binding material from the plastic to an elastic condition.

4. The herein described process, which consists in applying to a rotary surface, a binding material in the form of a dough like semi-solid plastic at the time of applica- 105 tion of such high cohesiveness and ad- 110 hesiveness as to be capable of penetrating around and between the natural fibres of the material to be treated, applying said coated surface with pressure to a fabric composed of unspun unwoven fibres and forcing por- 115 tions of said coating or binding material into the fabric and around and upon the individual fibres throughout the fabric, so as to coat the individual fibres without fill- 120 ing the interfibre spaces, and separating the impregnated fabric from the coated rotary surface so as to leave the adjacent surface of the fabric roughened, and portions of the surface fibres coated and upstanding so as to form bonds for a subsequent exterior coating.

5. The herein described process, which consists in applying to a rotary surface, a binding material in the form of a dough like semi-solid of such high cohesiveness and ad- 125 hesiveness as to be capable of penetrating around and between the natural fibres of the

material to be treated, applying said coated surface with pressure to a fabric composed of unspun unwoven fibres and forcing portions of said coating or binding material 5 into the fabric and around and upon the individual fibres throughout the fabric, so as to coat the individual fibres without filling the interfibre spaces, and separating the impregnated fabric from the coated rotary surface 10 face so as to leave the adjacent surface of the fabric roughened, and portions of the surface fibres coated and upstanding so as to form bonds for a subsequent exterior coating, treating the opposite face of the fabric 15 in like manner by means of a rotary surface coated with the binding material, and simultaneously treating the roughened previously treated surface of the fabric with pressure by a rotary surface free from binding material, to roll down the upstanding fibres and smooth the roughened surface thereof.

6. The herein described process, which consists in applying to a roller of a calender an adhesive coating of binding material comprising a rubber base plastic at the time of application, and made plastic by milling, and passing between said coated roller and an opposed roller, an unwoven fabric composed of unwoven unspun fibres to units 25 30 said fibres in said fabric.

7. The herein described process which consists in coating a roller of a calender with binding material plastic at the time of application having a rubber base, mixed with

sulphur, and rendered plastic by milling 35 without the addition of volatile liquid solvents, and passing between said coated roller and an opposed roller an unwoven fabric composed of unwoven, unspun fibres, to unite the fibres in the fabric, and then vul- 40 canizing the fabric.

8. The herein described process which consists in coating a roller of a calender with binding material plastic at the time of application having a rubber base mixed with sulphur and filling material, and rendered plastic by milling, and passing between said coated roller, and an opposed roller, under pressure, a non-woven fabric composed of unspun fibres to unite the fibres in the fabric 50 and carry the filling material with the other components of the binding material into the fabric.

9. The herein described process which consists in calendering an unwoven fabric composed of unspun fibres with a binding material in semi-solid form and plastic at the time of application, consisting of rubber mixed with sulphur and brought into plastic condition by milling, without the use of volatile solvents, to force said plastic binding material into the interfibre spaces of the plastic, and coat the fibres without completely filling the interfibre spaces.

In testimony whereof we affix our signatures.

HERMAN E. BROWN.  
JORDAN HOMER STOVER.